

## UNITED STATES PATENT OFFICE

2,129,666

## ESTERS OF METHACRYLIC ACID

Harold J. Barrett and Daniel E. Strain, Wilmington, Del., assignors to E. I. du Pont de Nemours & Company, Wilmington, Del., a corporation of Delaware

No Drawing. Application July 14, 1934,  
Serial No. 735,278

6 Claims. (Cl. 260—2)

The present invention relates to new compositions of matter, to methods for their preparation, and more particularly to the methacrylic acid esters of the alicyclic alcohols.

5 An object of the present invention is to provide new compositions of matter and a process for their preparation. A further object of the invention is to provide a new polymerizable composition of matter together with a process for its 10 polymerization. A still further object of the invention is to provide a process for the preparation of the methacrylic acid esters of the alicyclic alcohols which may be obtained by the ester interchange method of interacting a lower 15 alkyl ester of methacrylic acid with the alcohol in the presence of a suitable catalyst or by the reaction of the alcohol with a methacrylyl halide. Another object of the invention is to provide mixtures or interpolymers of the polymerized resin 20 with other polymerizable compounds of methacrylic and acrylic acids. Other objects and advantages of the invention will hereinafter appear.

There have been prepared in accord with this 25 invention valuable esters of methacrylic acid which have been found useful as prepared and even more valuable when polymerized. These compounds may be generally described as methacrylic acid esters of the alicyclic alcohols, such, for example, as tetrahydrofurfuryl alcohol, cyclo- 30 hexanol, decahydrobetanaphthol, decahydroalphanaphthol, alicyclic tetrahydrobetanaphthol, 1, 2, or 3-alkyl substituted cyclohexanols, naphthenyl alcohols, betacyclohexyl ethyl alcohol; the alkyl or aryl substituted tetra or decahydroalpha- 35 or beta-naphthols, such, for example, as aliphatic decahydrobetanaphthol, alphaphenyltetrahydrobetanaphthol; naphthanyl; abietyl alcohol and equivalent and homologous alcohols.

The following specific examples are furnished 40 to illustrate methods of preparing the new compositions of matter but it will be understood that the invention is not limited to the details therein given.

Example 1.—200 parts of cyclohexanol, 800 45 parts of methyl methacrylate, 450 parts of benzene, 48 parts of hydroquinone, and 15 parts of p-toluene sulfonic acid (tech.) (all parts are by weight) are mixed and warmed on the water bath until solution is complete. The solution was then 50 heated on an oil bath which was maintained at a temperature of 130—140° C. under a 48" fractionating column fitted with a condenser arranged for controlled reflux. The distillate, which consisted of a benzene-methanol binary, was collected at such a 55 rate that the temperature at the head of the column remained at 58—59°. Heating was continued until the temperature at the head of the column could not be maintained at 58—59°. The progress of the reaction was followed by measuring the amount of methanol in the distillate as shown by the portion that would dis-

ture at the head of the column remained at 58—59°. Heating was continued until the temperature at the head of the column could not be maintained at 58—59°. The progress of the reaction was followed by measuring the amount of methanol in the distillate as shown by the portion that would dissolve in water. The cold reaction mixture was neutralized and then washed and dried over a suitable desiccating medium. The solvents were removed from the dried product by fractional distillation, and the ester finally separated by fractionation under reduced pressure. A 62% yield of cyclohexyl methacrylate was obtained, which had a boiling point of 71—74° C. at 5 mm., a density at 20° C. of 0.959, and a 15 saponification number of 322, (theoretical 332).

Example 2.—The process of Example 1 was repeated with 800 parts of methyl methacrylate, 200 parts of tetrahydrofurfuryl alcohol, 700 parts of benzene, 50 parts of hydroquinone, and 5 parts of sulfuric acid (concentrated). The temperature of the oil bath was maintained at approximately 140—155° C. and after 16 hours a 44% yield of tetrahydrofurfuryl methacrylate was obtained having a boiling point of 81—85° C. at 4 20 mm., a density at 20° C. of 1.039, and a saponification number of 326, (theoretical 330).

Example 3.—The process of Example 1 was repeated with 330 parts of methyl methacrylate, 110 parts of decahydrobetanaphthol, 275 parts of 30 benzene, 20 parts of hydroquinone, and 10 parts of p-toluene sulfonic acid 4H<sub>2</sub>O. The temperature of the oil bath was maintained at approximately 125—145° C. and after 21 hours a 77% yield of decahydrobetanaphthyl methacrylate 35 was obtained, which had a density at 20° C. of 0.998.

Example 4.—128 parts of naphthenyl alcohols, 275 parts of methyl methacrylate, 225 parts of benzene, 20 parts of hydroquinone, and 2 parts of concentrated sulfuric acid were mixed and warmed on the water bath until solution was complete. The solution was then heated on an oil bath which was maintained at a temperature of 130—140° C. under a 48" fractionating column 45 fitted with a condenser arranged for controlled reflux. The distillate, which consisted of a benzene-methanol binary, was collected at such a rate that the temperature at the head of the column remained at 58—59°. Heating was continued until the temperature at the head of the column could not be maintained at 58—59°. The progress of the reaction was followed by measuring the amount of methanol in the distillate as shown by the portion that would dis-

solve in water. The cold reaction mixture was dried over a suitable desiccating medium, the solvents removed by fractional distillation and the resulting mixture fractionated under reduced pressure. An 86% yield of naphthene methacrylate was obtained, which had a saponification number of 234, and a density at 20° C. of 0.928.

Other methods may, of course, be employed for the preparation of the enumerated methacrylates, such, for example, as are disclosed in the copending applications of Barrett and Strain, Serial Nos. 735,274, 735,276, and 735,279 or by any of the well known esterification or ester interchange processes.

15 The methacrylates as prepared in accord with the examples are usually mobile liquids, but may sometimes be solids. The esters as thus produced are monomeric and may be polymerized, according to the invention, by means of heat, light 20 and/or a catalyst, e. g. as described for the polymerization of organic vinyl esters in British specification 15271/1914. Preferably a catalyst such as oxygen, ozone, an organic peroxide, an ozonide, etc. is employed. Other catalysts which 25 may be used include aluminum sulfate, boron fluoride, the mineral acids, e. g. hydrochloric and sulfuric acids as well as the organic acids, for example, acetic, methacrylic acids, etc., as well as the anhydrides and acid halides of such organic 30 acids; metal salts of fatty acids and resinic acids, e. g. cobalt linoleate and resinate, manganese oleate and rosin, etc. The polymerization may be effected in the presence or absence of a solvent for both monomer and polymer, or in the presence of 35 a solvent for both monomer and polymer, or in the presence of a solvent for the monomer and a non-solvent for the polymer, or the monomer may be emulsified and then polymerized. Preferably 40 polymerization is carried out at a moderate temperature, i. e. between 60-100° C., altho higher temperatures, such as, for example, 130° C., or higher, may be employed. The polymerization reaction is usually strongly exothermic and it may be necessary to control the temperature by cooling devices, the polymerization may be carried out in apparatus which may be or may not be provided with condensing devices or in suitable 45 pressure equipment.

As indicated, various methods may be employed 50 for polymerizing the monomeric esters of methacrylic acid and it has been found that the properties of the resins, the physical properties to a large extent and the chemical properties to a lesser extent, are altered considerably by the type 55 of polymerizing process utilized. The process described in the copending applications of D. E. Strain, Ser. Nos. 668,080 and 704,753, may be used, if desired.

Methods illustrating the polymerization of the 60 esters will now be described, but it will be understood that other suitable polymerizing processes may be employed.

Example 5.—100 parts (parts are given by weight) of cyclohexyl methacrylate monomer was 65 dissolved in 400 parts of methanol in a bottle provided with a stopper, then 1 part of powdered benzoyl peroxide added to this solution. After the benzoyl peroxide was all dissolved, 90 parts of water, insufficient to cause permanent turbidity, 70 was added. The bottle was securely closed and set in an oven at approximately 65° C. After the polymerization was complete in approximately 2 days, the mixture was allowed to cool. The product was filtered, washed with a little cold 75 methanol, and dried in a vacuum desiccator. The

polymer was obtained in 93% yield as a white coarse powder. The polymer is soluble in butyl acetate and toluene, and relatively insoluble in gasoline and acetone. It has a viscosity of 0.065 poise (5% solution in toluene at 25° C.) and is 5 compatible with nitrocellulose. The resin was placed in a disk shaped mold in which it was subjected to a temperature of 160° C. and a pressure of approximately 4000 pounds per square inch for approximately 15 minutes. A molded clear, 10 colorless, strong disk was obtained which softened at a temperature of 105° C. The compatibility with nitrocellulose was determined by dissolving an equal volume of a 5% toluene solution of the polymerized ester in a solution consisting of 15 20 parts of nitrocellulose and 380 parts of butyl acetate. The resulting solution was spread on a glass plate and allowed to dry at room temperature.

Example 6.—The polymerization process of 20 Example 5 was repeated using 110 parts of tetrahydrofurfuryl methacrylate monomer, 250 parts of methanol, 1 part of benzoyl peroxide, and 54 parts of water. After 3 days at 65° C. an 86% yield of the polymer as a fused, brittle, glassy mass 25 was obtained, which was recovered by decanting the liquid, removing the polymer from the bottle, and after cutting into small pieces drying in a vacuum desiccator. The polymer was relatively insoluble in butyl acetate, gasoline, acetone, and 30 toluene. The resin was placed in a disk shaped mold in which it was subjected to a temperature of 100° C. and a pressure of approximately 4000 pounds per square inch for approximately 15 35 minutes. A molded, slightly amber-colored disk was obtained which softened at a temperature of 60° C.

Example 7.—Undiluted decahydronaphthyl methacrylate monomer containing 1.9% benzoyl peroxide was heated to a temperature of 100° C. 40 After 2 days a 91% yield of polymer was obtained which upon extraction with methanol gave a gray, sandy-like powder. The polymer is soluble in butyl acetate, gasoline, and toluene, and relatively insoluble in acetone. It has a viscosity of 0.02 45 poise (5% solution in toluene at 25° C.). The resin was placed in a disk shaped mold in which it was subjected to a temperature of 125° C. and a pressure of approximately 4000 pounds per square inch for approximately 15 minutes. A 50 molded transparent, brown, brittle disk was obtained which softened at a temperature of 75° C.

Example 8.—Undiluted naphthene methacrylate monomer containing 1.6% benzoyl peroxide was heated to a temperature of 65° C. for 14 55 hours and at 100° for 24 hours. A 90% yield of the polymer was obtained as a brown, transparent, slightly soft and sticky fused mass. It is soluble in butyl acetate, gasoline, and toluene, and relatively insoluble in acetone. It has a 60 viscosity of 0.02 poise (5% solution in toluene at 25° C.), and is compatible with nitrocellulose which was determined as in Example 5.

Valuable products may be obtained by utilizing the polymers of the esters described herein 65 together with equivalents or homologues thereof admixed with other polymeric acrylic or methacrylic esters or other derivatives. Especially valuable products result if the monomeric esters are mixed and then polymerized. By this 70 method interpolymers having a wide range of characteristics are made. Due to the unique characteristics of methyl methacrylate polymer, which is a hard resin having a high melting point, its admixture with the polymeric esters of 75

methacrylic acids herein described or interpolymers thereof are particularly well adapted for many uses.

The polymerized esters of methacrylic acid, as well as mixtures or interpolymers thereof with other polymerizable compounds, are particularly well suited for thermoplastic molding. The monomer may be polymerized and/or reformed prior to placing in the mold and then may be molded in accord with the usual procedural steps employed, particularly in the molding of methyl methacrylate as described in the Rowland Hill Patent 1,980,483 of Nov. 13, 1934. The mold preferably is hot, prior to the introduction of the polymerization product, is then closed and the material so confined heated and pressed, the temperatures ranging from approximately 80-150° C., and pressures from 200 pounds per square inch upward are usually sufficient to give a suitably molded product. The presence or absence of plasticizers will, of course, alter considerably the molding conditions, and it is usually advantageous to have present plasticizers to alter the physical characteristics of the resulting product to fit the particular need for which the molded article is to be used.

The masses resulting from polymerization can immediately (i. e. in the state they have been obtained) be made into useful articles. It is possible to obtain the required articles if, for instance, the polymerization be carried out while the initial material is in a suitable mold, for instance one of steel or glass, so that the articles, for example, umbrella handles, fountain pen barrels, buttons, and the like, are obtained directly from the mold. Or, if desired the masses may be worked to the required shape by softening with suitable softeners or plasticizers in the presence of volatile solvents and after shaping, evaporating the solvent.

The polymerization products may be worked into the required shapes in various ways; for example, they can be softened and kneaded, rolled, compressed, drawn into wires, threads, or the like, or the masses can be mixed with additional substance and rolled into plates, or films, or they may be pressed into the required shapes, such as buttons, combs, and the like.

The solid masses can be worked by cutting, sawing, filing, or the like, whether they be obtained directly by polymerization, or after special treatment of the polymerized masses. These shaped articles may be polished, and parts connected together by smearing the faces to be connected with a suitable solvent, such as acetone, epichlorhydrin, or the corresponding methacrylic acid ester.

The polymerization product dissolved in a suitable solvent which may or may not be the monomer may be transformed into a useful article, e. g. films, by casting and then evaporating the solvent, or by extruding thru a suitable orifice into a precipitating bath or drying atmosphere. The polymer may be recovered from such solutions by precipitation with a suitable non-solvent for the polymer.

The properties of the resulting masses may be widely varied by modification with plasticizers, e. g. dibutyl phthalate, tricresyl phosphate, etc., drying, semi-drying, and non-drying oils, synthetic and natural resins, waxes, bitumens, cellulose derivatives, e. g. cellulose nitrate and ethyl cellulose, etc., pigments, fillers, and dyes, etc. Thus it is possible to produce, instead of hard glass-like masses, also soft and flexible masses.

Likewise, by the addition of suitable coloring means, it is possible to produce masses, or objects, having any desired color effects. The incorporation of the additions can be effected either before or during the polymerizing process, or the additions can be made to the already formed polymerization products in a suitable condition.

If the polymerization of an organic methacrylic acid ester be carried out in an incomplete manner, a syrupy solution of the polymerization product containing some unchanged methacrylic acid ester is obtained. This product can be utilized either directly or along with other solvents or diluents for the production of substances to be used for coating, painting or impregnating purposes; if, for instance, a porous substance such as wood, paper, textile fabric, artificial stone, or the like be coated with the said syrupy solution or be impregnated therewith, very resistant coatings and impregnations are obtained on completing the polymerization of the coating, painting or impregnation, for instance, by exposing the article to artificial or natural light, or by heating it, or by employing both light and heat. In this case a portion of the unchanged methacrylic acid ester in the syrupy solution may or may not be evaporated while another portion may be converted into the solid polymerization product. The articles thus treated have imparted to them a very high resistance to external influences, e. g. resistance to water, acids, alkalies, and atmospheric changes.

The syrupy mass can be mixed with comminuted matter, such, for instance, as ground cork, or ground wood, fibrous substances, mineral fillers, or the like, and the mixture be made into the proper shape and the unchanged methacrylic acid esters in the articles be converted by suitable polymerization into the solid final product.

It is also possible to start from solid, semi-solid, or plastic polymerization products of the methacrylic acid esters, these being softened by heating them by themselves, or with suitable solvents, and using them in their softened state. On cooling or on the evaporation of the diluent that may still be present, the product is converted into the solid lacquer-form.

It is obvious that mixtures of various polymerized methacrylic acid esters can be used for lacquering, painting, or impregnating in accordance with this invention. It is likewise obvious that the wholly or partly polymerized esters can be mixed with suitable additional substances to modify the properties of the lacquering, painting, or impregnating materials in any desired manner. As additions of this kind oils should be mentioned (such, for instance, as castor oil) dyes, powdered substances (such as zinc oxide), camphor, camphor substitutes, and the like.

In accordance with this invention it is possible to obtain valuable products if the said polymers be dissolved or softened in suitable solvents and then be converted again to the solid state. The products thus obtained may be used for purposes for which cellulose esters have hitherto been used, namely, as substitutes for horn, amber, artificial resins, lacquers, for impregnating purposes and also for the production of films, interlayer for safety glass, pressure adhesives, artificial threads, and the like.

The products thus formed have the advantage over products made from nitrocellulose in being less inflammable. By the addition of suitable agents, the strength and hardness of the products

may be modified within wide limits so that it is possible to manufacture both hard, horn-like substances and soft and more pliable products. The products may also be modified by varying the 5 conditions of the polymerization.

The monomer may be polymerized in the presence of a solvent and the solution used as such or the polymer recovered from the solution by evaporation or precipitation methods. In many 10 cases, however, it is more profitable to use an amount of solvent insufficient to produce a freely flowing solution, so that soft plastic masses are obtained which can be pressed, kneaded, rolled or drawn into shape, or formed into blocks, plates, 15 or films.

Plasticizers or other modifying agents may be added to the monomer prior to polymerization or directly to the polymerized product, it being generally desirable to employ a plasticizer which is 20 soluble in the polymer and the monomer, although it is not essential that the dual solubility characteristics be present. Thus, plasticizers or softening agents, such as, for example, camphor; phthalates, such as ethyl, propyl, isopropyl, butyl, 25 isobutyl, cyclohexyl, methyl cyclohexyl, or benzyl phthalate or phthalates of the mixed types such as cyclohexyl butyl, benzyl butyl or butyl lauryl phthalate; esters of other dibasic acids, such as the ethyl, propyl, isopropyl, butyl, isobutyl, cyclo- 30 hexyl, methyl cyclohexyl or benzyl esters of succinic, fumaric, tartaric, adipic and sebacic acids; esters of monobasic acids, such as the butyl, isobutyl, cyclohexyl, methyl cyclohexyl, benzyl or lauryl esters of lauric, laevulinic, benzoic, benzoyl 35 propionic and benzoyl benzoic acids; esters of polyhydric alcohols, e. g. glycol and glycerol, such as glycol benzoate, glycol laevulinate, triacetin, tripropionin and tributyrin; substituted toluene sulphonamides, such as ethyl paratoluene sul- 40 phonamide; substituted amides, such as tetraethyl phthalamide, tetrabutyl succinamide, tetrabutyl adipamide, tetraethyl phthalamide; hydrocarbons, such as dixylyl ethane; halogenated hydrocarbons, such as chlorinated diphenyls and 45 dichlorodibenzyl; ether compounds such as dicresoxy ethyl ether; and drying, non-drying, or semi-drying oils, such as castor oil, cotton seed oil, linseed oil, and the like. These additions also facilitate later mechanical treatment, as cutting, sawing, and polishing.

The polymerized esters, mixtures of the polymerized esters with dissimilar polymerizable esters or other polymerizable compounds of methacrylic or acrylic acids, or vinyl compounds, or 50 interpolymers of the esters with such other compounds, may be used advantageously as safety glass interlayers. These polymerized esters, mixtures thereof, or interpolymers thereof may be

plasticized or otherwise modified as desired. The compositions may be compounded with glass in an unpolymerized, partially polymerized, or completely polymerized condition. When compounding the safety glass with the unpolymerized or 5 partially polymerized compositions, the polymerization may be effected by subjecting the sandwich of glass and compound to suitable application of light and/or heat.

From a consideration of the above specification 10 it will be realized that various changes may be made in the process or product without departing from the invention or sacrificing any of its advantages.

We claim:

1. The polymeric methacrylic acid ester of an alcohol selected from the group consisting of an alicyclic alcohol and tetrahydrofurfuryl alcohol, in which there is no branch-chain substitution on the carbon atom adjacent to the carbinol group, 20 prepared by heating the monomeric ester to a temperature of from 60 to 100° C., in the presence of benzoyl peroxide.

2. The polymeric cyclohexyl methacrylate prepared by heating monomeric ester to a temperature of from 60 to 100° C., in the presence of benzoyl peroxide.

3. The polymeric tetrahydrofurfuryl methacrylate prepared by heating the monomeric ester to a temperature of from 60 to 100° C., in the 30 presence of benzoyl peroxide.

4. The polymeric decahydrobetanaphthol methacrylate prepared by heating the monomeric ester to a temperature of from 60 to 100° C., in the presence of benzoyl peroxide.

5. The molding composition comprising the polymeric methacrylic acid ester of an alicyclic alcohol selected from the group consisting of an alicyclic alcohol and tetrahydrofurfuryl alcohol, in which there is no branch-chain substitution on the carbon atom adjacent to the carbinol group, 40 prepared by heating the monomeric ester to a temperature of from 60 to 100° C., in the presence of benzoyl peroxide.

6. The interpolymer of a methacrylic acid ester 45 of an alcohol selected from the group consisting of an alicyclic alcohol and tetrahydrofurfuryl alcohol, in which there is no branch-chain substitution on the carbon atom adjacent to the carbinol group, and a polymerizable derivative of an acid selected from the group consisting of acrylic acid and methacrylic acid, which interpolymer is prepared by heating a mixture of the monomeric compounds to a temperature of from 60 to 100° C., in the presence of benzoyl peroxide.

HAROLD J. BARRETT.  
DANIEL E. STRAIN.